

## UNITED STATES PATENT OFFICE

2,138,014

## PREPARATION OF VISCOSE SIRUP

George A. Richter, Berlin, N. H., assignor to  
 Brown Company, Berlin, N. H., a corporation  
 of Maine

No Drawing. Application May 1, 1937,  
 Serial No. 140,222

4 Claims. (Cl. 260—100)

This invention relates to the preparation of viscose and has for its general objective the economical preparation of viscose sirup such as is suitable for the manufacture of artificial silk, 5 films, and regenerated cellulose products.

In accordance with the present invention, viscose sirup is prepared by the xanthation of alkali cellulose comprising a blend of acid-preliberated cellulose pulp of the nature of sulphite pulp and 10 alkali-preliberated cellulose pulp of the nature of kraft and soda pulps, although kraft or similar alkali-preliberated pulps do not by themselves yield viscose sirups satisfactory for the manufacture of artificial silk, films, and similar 15 ultimate products, the blending therewith of upwards of about 25% sulphite or similar acid-preliberated pulp, based on the weight of the blend, preparatory to xanthation makes possible the obtainment of viscose sirups quite satisfactory for manufacture into such ultimate products.

The advantages to be realized from the practice hereof may perhaps be best appreciated by 25 considering the results realized when acid-preliberated wood pulp, such as sulphite, and alkali-preliberated wood pulp, such as kraft, separately undergo the usual viscose-making operations. These operations involve dipping sheets of the 30 pulp in strong caustic soda solution, pressing the sheets to form alkali cellulose of appropriate solution content, grinding the sheets into crumbs or shreds, aging the crumbs, and xanthating the crumbs by tumbling them in a slowly revolving drum in the presence of carbon bisulphide vapor. 35 When xanthate crumbs are thus prepared from sulphite pulp, it is found that they dissolve readily and substantially completely in dilute caustic soda solution to yield a cellulose xanthate solution or viscose sirup suitable for the manufacture 40 of artificial silk. When, on the other hand, xanthate crumbs are similarly prepared from kraft pulp, it is found that they are resistant to substantially complete dissolution in dilute caustic soda solution and that the resulting viscose 45 sirup contains a substantial residue of fiber fragments or gelatinized particles bespeaking incomplete xanthation of the pulp and inutility of the viscose sirup for the manufacture of artificial silk. The fact is that in terms of filterability or 50 capacity for filtration the viscose sirup prepared from sulphite pulp generally displays a filterability of about 1500 to 1800 cubic centimeters as compared with a filterability of only about 100 to 200 cubic centimeters in the case of viscose 55 sirup prepared under similar conditions from a

kraft base pulp. The filterability test employed herein is performed under standard conditions with a filter pad of standard structure and area; and the volume of viscose sirup filtrate delivered by the pad before it becomes plugged with fiber 5 fragments or gelatinized particles present in the sirup is taken as the filterability of the sirup. When viscose sirup was prepared pursuant to the invention hereof from a blend consisting of about equal proportions of the same sulphite pulp and 10 the same kraft pulp productive of the viscose sirups whose filterabilities have just been given, it was found that the viscose sirup had a filterability of about 1400 to 1600, that is, partook in surprisingly large measure of the quality of filterability possessed by the viscose sirup prepared from the sulphite pulp alone, despite the fact that the sulphite pulp and the kraft base pulp had approximately the same solution viscosity 15 as measured by the usual cuprammonium cellulose solution test.

While it is difficult to account for the results realized by the practice hereof, yet they may perhaps be explained by what happens when alkali-cellulose crumbs are prepared from sulphite pulp alone and from kraft pulp alone. Thus, alkali-cellulose crumbs prepared from sulphite pulp are characterized by a fluffy or open structure permitting ready and substantially uniform access of carbon bisulphide vapor throughout such structure. Per contra, alkali-cellulose 25 crumbs prepared from kraft pulp are of relatively dense, coarse, and stringy texture and, because of non-uniform access of carbon bisulphide vapor to their interiors, yield dense, 30 soggy xanthate crumbs whose resistance toward sufficiently complete dissolution in dilute caustic soda solution has already been mentioned. It is evidently the case that when the alkali-cellulose 35 product of sulphite pulp and the alkali-cellulose product of kraft pulp are ground simultaneously into crumbs, the resulting mass or blend of 40 crumbs is rendered sufficiently voluminous or distended so that when the mass is put into a slowly rotating drum and xanthated by exposure 45 to carbon bisulphide vapor, the vapor can penetrate into and throughout the distended or voluminous mass with sufficient rapidity and uniformity to yield xanthate crumbs of the desired 50 substantially complete solubility in dilute caustic soda solution to conduce to viscose sirup suitable for manufacture into artificial silk.

A typical example of procedure in conformity with the invention hereof may involve the use of 55 bleached sulphite pulp and bleached kraft pulp

whose compositions, other than pentosan content, may be substantially similar. Thus, the compositions of the two bleached pulps may be those appearing in the table below:

|                      | Sulphite  | Kraft     |
|----------------------|-----------|-----------|
| Alpha cellulose..... | 88 to 89% | 88 to 89% |
| Viscosity.....       | 2 to 4    | 2 to 4    |
| Pentosans.....       | 2.5 to 4% | 5 to 9%   |

Both the sulphite and kraft pulp may be derived from spruce or other coniferous wood and may be used in the form of drier sheets or pulpboards as ordinarily. Equal portions of such pulps may be steeped in strong caustic soda solution to form alkali cellulose, as by stacking sheets of the sulphite pulp alternately with sheets of the kraft pulp and submersing the stack in the solution with the sheets in upstanding position. The stack may thus be put into the usual steeping press wherein the sheets may be thoroughly soaked or saturated with caustic soda solution of about 18% strength at about 20° C. for about 3 hours. Excess soaking solution may be drained from the press and the stack of soaked sheets then pressed to a solution to pulp ratio of about 3 to 1, based on the original weight of the sheets. The pressed sheets may then be taken from the stack and disintegrated into soda cellulose crumbs in the usual grinders, wherein the grinding of a mass of, say, 200 pounds cellulose content may be effected for a period of about 3 hours at a temperature of about 20° to 24° C. The resulting soda-cellulose crumbs, which are of fluffy open structure, may then be aged at about 20° C. for about 70 hours, whereupon they may be charged into the usual rotary xanthating drum into which carbon bisulphide in the form of vapor may be progressively delivered in the amount of, say, about 35%, based on the dry weight of original cellulose, for a period of about 3 hours while the mass in the drum is kept at a temperature of about 25° C. At the end of such period, the resulting porous mass of orange-colored xanthate crumbs may be sluiced from the xanthating drum into a dissolving tank wherein the xanthate crumbs may be mixed with dilute caustic soda solution predetermined as to volume and causticity to yield viscose sirup of about 7.5% cellulose content and about 6.5% causticity based on the weight of the sirup. The desired substantially complete dissolution of the xanthate crumbs may be had after mixing intimately with the dilute caustic soda solution at about 15° to 20° C. for about 3 to 4 hours. The resulting viscose sirup is a thick clear liquid practically free from unxanthated or incompletely xanthated residues and hence of good filterability. Upon being deaerated, as usual, such viscose sirup is spinnable into artificial silk of strength and color qualities comparing favorably with artificial silks as heretofore manufactured by the viscose process from sulphite pulp or cotton linters. It is possible to depart in various respects from the particular example hereinbefore given. Thus, rather than mixing sheets of the sulphite and kraft pulp while they are being dipped or soaked in the strong caustic soda solution, it is possible to dip or soak sheets consisting of a blend of the two pulps; and it is also possible to dip or soak the sulphite pulp sheets in strong caustic soda solution independently of the kraft pulp sheets, provided that the resulting sheets of soda cellulose are ground together at the same time so that

crumbs or alkali cellulose produced from the sulphite pulp sheets are substantially uniformly blended with the crumbs of alkali cellulose produced from the kraft pulp sheets, thereby providing an alkali-cellulose blend or mass of the appropriate fluffiness or voluminous structure for the xanthating reaction. When sheets of sulphite pulp and sheets of kraft pulp are dipped or soaked in separate caustic soda solutions, it is possible to operate under dipping conditions, i. e., time and temperature of dipping and causticity of dipping solution, different for each of the two types of sheet and designed to promote the formation of the best kind of alkali cellulose from each type of sheet. Thus, it may be desirable to furnish for the kraft pulp sheets a dipping or soaking solution of much greater causticity, namely, of much greater than 18% strength, and/or to maintain such sheets in a solution at lower temperature and/or for a longer period of time than in the case of the sulphite pulp sheets. In this latter connection, it should be understood that the stronger the dipping solution, the lower the temperature at which it is used, and the longer the dipping period, the greater is the reactivity of the resulting soda cellulose in the subsequent xanthating reaction.

The invention hereof affords the important advantage that it makes available for satisfactory use in the viscose-rayon process the various alkali-preliberated wood pulps heretofore found unsuitable for viscose-rayon manufacture, including alkali-preliberated pulps derived from various resinous or deciduous woods which, although lending themselves nicely to low-cost pulping by the soda, kraft, and other alkaline fiber-liberating processes, do not respond to pulping in acid sulphite or similar acid fiber-liberating liquors. The expressions "alkali-preliberated cellulose pulp" or "alkali-preliberated wood pulp" used herein are meant to include wood pulps derived from both coniferous and deciduous woods by kraft, so, or equivalent alkaline pulping liquors and to include such pulps in unbleached, semi-bleached, bleached, unrefined, or refined conditions, as all such pulps may advantageously undergo the process hereof. Insofar as concerns unbleached or semi-bleached alkali-preliberated pulps, it will, of course, be appreciated that their utility herein extends to the making of artificial silk or other regenerated cellulose products wherein the color factor is of no particular materiality but wherein the factor of strength is of importance. So far as concerns the factor of strength, regenerated cellulose products resulting from the process hereof, when the alkali-cellulose blends contain alkali-cellulose produced from unbleached or semi-bleached alkali-preliberated cellulose pulps, exhibit a strength superior to that of the usual regenerated cellulose products. The utility of the instant invention resides more especially in the making of viscose sirups of a cellulose content and causticity each ranging from about 6% to 10%, since it is the making of viscose sirup of such composition from alkali-preliberated cellulose pulp that has presented the problem solved in such a simple and satisfactory way by the instant invention.

I claim:

1. A process of making viscose, which comprises producing an alkali-cellulose blend from acid-sulphite-preliberated cellulose pulp and alkali-preliberated cellulose pulp in approximately equal proportions to not less than about 25% of said first-named pulp relative to the total cellu-

lose content of said alkali-cellulose, xanthating the alkali-cellulose blend, and dissolving the resulting cellulose xanthate to form viscose.

2. A process of making viscose, which comprises grinding into crumbs sheets of alkali-cellulose whose cellulose includes both acid-sulphite-preliberated cellulose pulp and alkali-preliberated cellulose pulp in approximately equal proportions to not less than about 25% of said first-named pulp relative to the total cellulose content of said alkali-cellulose, xanthating the crumbs, and dissolving the xanthated crumbs to form viscose sirup.

3. A process of making viscose, which comprises grinding into crumbs sheets of alkali-cellulose comprising at least two different cellulose components, one of said components being acid-sulphite-preliberated wood pulp and the other of said components being alkali-preliberated wood pulp of the nature of kraft and soda pulp in

such proportions as to yield a blend of alkali-cellulose crumbs whose cellulose content is furnished to the extent of about 25% to 50% by said first-named pulp, xanthating the blend, and dissolving the resulting cellulose xanthate to form 5 viscose.

4. A process of making viscose, which comprises forming alkali-cellulose from sheets of acid-sulphite-preliberated cellulose pulp and from sheets of alkali-preliberated cellulose pulp, 10 simultaneously grinding into crumbs the sheets of alkali-cellulose produced from both types of pulp in such proportions as to yield a blend of alkali-cellulose crumbs whose cellulose content is furnished to the extent of about 25% to 50% 15 by said first-named pulp, xanthating the blend of alkali-cellulose crumbs, and dissolving the xanthated crumbs to form viscose sirup.

GEORGE A. RICHTER. 20